

## UNITED STATES PATENT OFFICE

ARTHUR B. BROWN AND FREDERICK W. SULLIVAN, JR., OF WHITING, INDIANA, AS  
SIGNORS TO STANDARD OIL COMPANY, OF WHITING, INDIANA, A CORPORATION OF  
INDIANA

## MANUFACTURE OF NONDETONATING MOTOR FUELS

No Drawing.

Application filed November 12, 1925. Serial No. 68,706.

The present invention relates to the improvements in the production of non-detonating fuels particularly intended for use in internal combustion engines such as automobile engines and to the production of organic nitrogen compounds and will be fully understood from the following description, in which specific examples of such fuels and their manufacture are set forth by way of illustration.

In accordance with this invention, we subject a hydrocarbon oil product, preferably heavier than gasoline, to conversion conditions of temperature and pressure in the presence of nitrogen compounds which may be regarded as substituted ammonias. In subjecting the initial material to such conditions of pressure and temperature, distillation of lighter products of conversion in the gasoline range of boiling points may be accomplished simultaneously by a distillation operation, or such products may be removed from the reaction chamber after the desired reaction has been completed. The resulting product having the gasoline range of boiling points and containing the nitrogenous products of reaction may be employed directly as a motor fuel, or may be admixed with ordinary gasolines as found on the market in suitable proportions to produce the desired degree of anti-knock action.

The proportion of the nitrogenous compounds employed may be varied within wide limits. In general, we find it advisable to use from 2 to 15% by weight of the nitrogenous compounds. As examples of nitrogenous compounds which we have employed, the following are enumerated: ammonia; urea; ammonium carbonate; guanidine; and dicyandiamide.

In operating in accordance with the present process, a suitable high boiling hydrocarbon oil, for example, gas oil, may be heated under pressure to conversion temperatures of, say 700° F. or higher, and preferably 750° to 850° F., suitably in a vessel adapted to retain high pressure. Sufficient pressure is employed, say 4 to 5 atmospheres or higher, to maintain the hydrocarbon oil stock treated substantially in liquid phase. The

conditions of pressure and temperature are maintained for a suitable period, say two hours or longer, to effect a substantial conversion of the oil treated into products of the gasoline range of boiling points, there being 55 a conversion into such products exceeding 3%. Preferably the process is carried to a much further degree, the length of the operation being continued until a conversion of at least 20% into products of the gasoline range 60 of boiling points has been secured. When the digestion operation has been completed, the products are subjected to distillation for the removal of those in the gasoline range 65 of boiling points. With substantially all of 65 the substituted ammonia compounds employed, this gasoline cut of the product is found to contain an appreciable quantity of nitrogen, in excess of 0.1%. The resulting gasoline product may be employed as a non- 70 detonating fuel or may be admixed with ordinary gasolines to improve their anti-knock qualities.

Thus, by operating in this manner, employing urea, a gasoline-like product was obtained which, when mixed with twice its volume of a typical mid-continent gasoline, resulted in a fuel equivalent in its anti-knock qualities to a mixture of the same gasoline and benzol containing 23% of benzol. The 80 organic nitrogenous product of reaction appears to be cyclic in character, of the nature of pyridine. Operating similarly, employing other compounds, such as ammonium carbonate, guanidine, dicyandiamide, etc., similar results are secured. Thus, with dicyandiamide, the benzol equivalent of the resulting motor fuel, when mixed with twice its volume of a mid-continent gasoline, is 16 to 20%. 85

Although the invention has been described in connection with a digestion operation, it may be carried out also in connection with a pressure distillation operation or with a continuous type of digestion operation. For 95 example, the heavy hydrocarbon oil with which the nitrogenous compound is admixed may be subjected to distillation under pressure of 4 to 5 atmospheres upwardly, and preferably of 100 to 350 pounds. In such an 100

operation, vapors of products heavier than the desired product may be cooled and the resulting condensate reflux to the material undergoing distillation, as is customary in pressure distillation of heavy oils for the production of gasoline. The mixture of heavy hydrocarbon oil and the nitrogenous compound may also be passed in continuous flow through a heating zone to be brought to the desired conversion temperature and maintained at such temperature and under pressure while flowing at a slower rate through a chamber or receptacle in which further conversion and reaction may take place.

15 We claim:

1. The method of producing non-detonating fuel which comprises subjecting a high boiling hydrocarbon oil to conversion temperatures while under pressure in the presence of a nitrogenous organic compound of substituted ammonia type, thereby producing cyclic nitrogen compounds in the oil, and distilling from the reaction mass a fuel product in the gasoline range of boiling points.
2. The method of producing a non-detonating fuel which comprises heating a high boiling hydrocarbon oil to conversion temperature at which low boiling oils are produced therefrom while under pressure in the presence of an organic compound containing an amino group, thereby producing cyclic nitrogen compounds in the oil.
3. A method of producing a non-detonating fuel which comprises heating a high boiling hydrocarbon oil to temperatures at least 700° F. while under pressure in the presence of a urea.
4. A method of producing a non-detonating fuel which comprises heating a high boiling hydrocarbon oil to temperatures at least 700° F. while under pressure in the presence of dicyandiamide.
5. A method of producing a non-detonating fuel which comprises heating a high boiling hydrocarbon oil to temperatures at least 700° F. while under pressure in the presence of guanidine.

ARTHUR B. BROWN.  
FREDERICK W. SULLIVAN, JR.